

## UNITED STATES PATENT OFFICE

2,417,405

## ARTIFICIAL LEATHER PRODUCT

Felix J. Bellac, New York, N. Y.

No Drawing. Application April 6, 1944,  
Serial No. 529,835

3 Claims. (Cl. 117—73)

1

This invention relates to artificial leather products and more particularly to artificial leather products comprising as a base a rubber coated fabric provided with nitrocellulose containing coatings.

It has been known in the art to manufacture artificial leather products by applying to a fabric base, for example a cotton fabric, suitable nitrocellulose-containing coatings. It has also been suggested to apply a nitrocellulose lacquer, as a finishing coating, to a rubber coated fabric. However, the results hitherto obtained were not satisfactory particularly because a sufficiently strong, durable and uniform connection between the rubber coated base and the nitrocellulose-containing coatings was not obtained. No satisfactory patent leather products could be, therefore, hitherto produced on a rubberized fabric base.

The main object of the present invention is to provide an artificial leather product or patent leather of the above mentioned type, in which the fabric base consists of a rubber coated fabric, and the plastic surface layers consist of nitrocellulose containing coatings which are in durable, uniform and homogeneous connection with said rubber coated fabric base.

Another object of my present invention is to provide an intermediate nitrocellulose coat which firmly and uniformly adheres to a rubberized fabric base and forms a uniform and homogeneous connection with nitrocellulose containing top coats or finishing coats applied to said intermediate coat.

It is also an object of this invention to provide a nitrocellulose lacquer composition, which can be applied as a coat to textile fabrics and forms a firm, durable and homogeneous connection with said fabrics.

Other objects and the advantages of my invention will be apparent to those skilled in the art from the appended claims and the following specification which describes, by way of example, some preferred embodiments of the invention.

I have found that cellulose nitrate containing coatings forming a firm, durable and homogeneous coat or finish on rubberized fabric may be obtained by first applying to the rubber coated fabric an intermediate nitrocellulose coating of the type described hereinafter, and then applying to said intermediate coating one or more coats of customary nitrocellulose lacquers. According to my invention said intermediary nitrocellulose coating is obtained by using a solution containing cellulose nitrate, a synthetic resinous substance compatible with cellulose nitrate, pigments and plasticizers for cellulose nitrate and said synthetic resinous substance, in the presence of a relatively small amount of butyl stearate, and suitable diluents. In these solutions, as solvents,

2

for example, esters, ethers and ketones, such as amyl acetate, ethyl acetate, butyl acetate and acetone may be used. The synthetic resinous substances added to the cellulose nitrate solution are 5 alkyd resins obtained from one or more polyvalent alcohols, such as glycerine, one or more polybasic acids, such as phthalic acid, phthalic anhydride, adipic acid, succinic acid, and one or more drying oils and/or drying oil acids with or 10 without the addition of one or more further modifying agents, such as natural or synthetic resinous materials. It is to be understood that in the present specification and the appended claims the term "alkyd resin" is used to denote and include resins resulting from the interaction of the 15 above mentioned ingredients and compatible with nitrocellulose. As examples of the plasticizers, dibutylphthalate, dibutylsebacate, tributylphosphate, tricresylphosphate, blown castor oil, and 20 raw or blown rapeseed oil, may be mentioned. I have found, however, that the use of certain resinous substances, which are capable of acting as plasticizers, give particularly good results. Such resinous substances are the materials sold under 25 the trade-name "paraplex." These materials may be used in mixture with the alkyd resin or resins or instead of the alkyd resins. Mixtures of several plasticizers may also be used. In order to obtain a satisfactory intermediate coating, i. e., 30 a coating which forms a permanent, homogeneous and uniform connection with the rubberized fabric, and in which the nitrocellulose and other film-forming ingredients form a durable, homogeneous blend, I add a relatively small amount, 35 i. e., 2-5%, preferably about 3% by weight of butylstearate to the nitrocellulose-resin solution. As examples of the diluting agents used in preparing this solution, alcohols and hydrocarbons, such as denatured ethyl-alcohol and solvent 40 naphtha may be mentioned. Instead of the butyl stearate a mixture of butylstearate with Venetian turpentine resin may also be used.

I have further found that the addition of 45 certain organic compounds acting as interfacial tension reducing agents facilitates the formation of a strongly and uniformly adhering coating on the rubberized fabric base, and results in particularly homogeneous, durable products. The use of di-octyl sodium sulfosuccinate in an 50 amount of 0.1-0.5% (based upon the total weight of the nitrocellulose solution) has been found very useful.

After the application of the above described 55 first or intermediate coat to the rubberized fabric base, the coat is dried, the dried material is cured, and may then be provided with one or more nitrocellulose coatings or finishes as known in the manufacture of artificial leather or patent leather products. For example, the compositions described in my prior Patent No. 2,326,-

992, patented August 17, 1943, may be used with advantage. These coating compositions consist of nitrocellulose and plasticizers dissolved in a mixture of solvents and diluents, with or without the addition of pigments.

*Example I.*—A solution to be applied to a rubberized fabric as an intermediate coat consists of the following ingredients:

|                                                                                                                                            | Per cent |
|--------------------------------------------------------------------------------------------------------------------------------------------|----------|
| Cellulose nitrate (a mixture of equal parts of wet nitrocellulose of 5-6 seconds viscosity and wet nitrocellulose of 30 seconds viscosity) | 15-30    |
| A solvent consisting of 20-30% of ethyl acetate and 80-20% of acetone                                                                      | 15-30    |
| Dibutylphthalate                                                                                                                           | 3-8      |
| Alkyd resin A                                                                                                                              | 12-22    |
| Black paste                                                                                                                                | 5-10     |
| Denatured alcohol                                                                                                                          | 10-30    |
| Butylstearate (based on the total weight of the above ingredients)                                                                         | 3        |

The alkyd resin A used in the above composition was the reaction product of 12 parts by weight of glycerol, 14 parts by weight of phthalic anhydride, 55 parts by weight of linseed oil acids and 18 parts by weight of rosin.

After applying a coating of the above composition to said rubberized base, and drying the coated base, a top coat is provided by applying a lacquer of the composition described in one of the examples of my above mentioned prior Patent No. 2,326,992.

*Example II.*—A composition consisting of

|                                                                  | Parts by weight |
|------------------------------------------------------------------|-----------------|
| The nitrocellulose as used in the intermediate coat of Example I | 50              |
| Acetone                                                          | 50              |
| Ethylacetate                                                     | 25              |
| Dibutylphthalate                                                 | 10              |
| "Paraplex Reg. 2"                                                | 15              |
| The alkyd resin known under the trade-name "Aroplaz 930"         | 20              |
| Black paste                                                      | 25              |
| Denatured alcohol                                                | 25              |
| Butylstearate                                                    | 5               |

is applied as the intermediate coat to a rubberized fabric. The top coat applied to the intermediate coat may have the same composition as in Example I.

*Example III.*—The intermediate coat to be applied to a rubberized fabric base is produced from a composition consisting of the following ingredients:

|                                                                  | Parts by weight |
|------------------------------------------------------------------|-----------------|
| The nitrocellulose as used in the intermediate coat of Example I | 50              |
| Acetone                                                          | 50              |
| Ethylacetate                                                     | 25              |
| Dibutylphthalate                                                 | 10              |
| "Paraplex Reg. 2"                                                | 35              |
| Black paste                                                      | 25              |
| Denatured alcohol                                                | 25              |
| Butyl stearate                                                   | 5               |
| Di-octyl sodium sulfosuccinate                                   | 1.0             |

The top coat on this intermediate coat is produced from a composition consisting of the following ingredients:

|                                               | Parts by weight |
|-----------------------------------------------|-----------------|
| Nitrocellulose 30 ctpcs                       | 50              |
| Nitrocellulose $\frac{1}{4}$ second viscosity | 50              |
| Dibutylphthalate                              | 25              |
| Butanol                                       | 30              |
| Blown rapeseed oil                            | 15              |
| Solvent naphtha                               | 15              |

*Example IV.*—A composition consisting of

|                                                                                                         | Per cent |
|---------------------------------------------------------------------------------------------------------|----------|
| Nitrocellulose as used in Example I                                                                     | 15-30    |
| A solvent consisting of 10% ethyl acetate, 35% of butyl acetate, 5% of amyl acetate, and 50% of acetone | 15-30    |
| Dibutyl phthalate                                                                                       | 3-8      |
| Alkyd resin B                                                                                           | 12-22    |
| Black paste                                                                                             | 5-10     |
| Denatured alcohol                                                                                       | 10-30    |
| Butyl stearate                                                                                          | 3        |

is used for producing an intermediate coat on a rubberized fabric base. The alkyd resin B used in this composition was produced from 17 parts by weight of glycerol, 27 parts by weight of phthalic anhydride and 55 parts by weight of linseed oil acids. The top coat on this intermediate coat may be produced from the top coat lacquer described in Example I.

Instead of the above described alkyd resin B, a resin formed from 11 parts by weight of glycol, 7.5 parts by weight of phthalic anhydride, 65 parts by weight of linseed oil acids and 15 parts by weight of rosin may also be used.

*Example V.*—A composition consisting of

|                                                                  | Parts by weight |
|------------------------------------------------------------------|-----------------|
| The nitrocellulose as used in the intermediate coat of Example I | 50              |
| Acetone                                                          | 50              |
| Ethylacetate                                                     | 25              |
| Dibutylphthalate                                                 | 10              |
| "Paraplex Reg. 2"                                                | 15              |
| Alkyd resin C                                                    | 20              |
| Pigment paste                                                    | 25              |
| Denatured alcohol                                                | 25              |
| Butylstearate                                                    | 5               |

is applied as the intermediate coat to a rubberized fabric. The coated fabric is dried and cured and a top coat of the following composition is then applied to the intermediate coat:

|                                             | Parts by weight |
|---------------------------------------------|-----------------|
| Nitrocellulose 30-35 ctpcs                  | 60              |
| Nitrocellulose $\frac{1}{4}$ sec. viscosity | 40              |
| Dibutylphthalate                            | 25              |
| Butanol                                     | 20              |
| Solvent naphtha                             | 40              |
| Blown castor oil                            | 15              |

The alkyd resin C used in the above composition was obtained from 10 parts by weight of glycerol, 3.5 parts by weight of phthalic anhydride, 80 parts by weight of linseed oil acids and 6.5 parts by weight of rosin.

*Example VI.*—A composition consisting of

|                                                              | Parts by weight |
|--------------------------------------------------------------|-----------------|
| Nitrocellulose as used in the intermediate coat of Example I | 50              |
| Acetone                                                      | 50              |
| Ethylacetate                                                 | 25              |
| Dibutylphthalate                                             | 10              |
| Aroplaz 930                                                  | 20              |
| Pigment paste                                                | 25              |
| Denatured alcohol                                            | 20              |
| Di-octyl sodium sulfosuccinate                               | 1               |
| Butyl stearate                                               | 5               |

is applied as an intermediate coat to a rubberized fabric. The top coat applied to the intermediate coat may have the same composition as in Example V.

I have found that by using the above described compositions containing nitrocellulose and a synthetic resin of the above described type together

with butylstearate, very satisfactory products are obtained, in which the coatings applied to the rubberized fabric strongly and uniformly adhere thereto, and which represent flexible, durable artificial leather or patent leather products of excellent properties and appearance.

It is to be understood that in the present specification and the appended claims the terms "intermediate coat" and "top coat" denote coatings which are obtained in a manner well known per se to those skilled in the art by the subsequent application of several layers—for example 2-5 layers—to the base to be coated. Thus, my "intermediate coat" may be obtained by applying a first layer of the compositions described above, and then applying several further layers to the first layer. Similarly, the "top coat" described in my examples is also obtained by the subsequent application of several layers.

I have found it advantageous to add to the composition used in the first layer of the top coat, i. e., in the layer contacting the intermediate coat, a certain amount of aroplaz or paraplex. Aroplaz 930 or paraplex reg. 2 may be added to said composition in an amount of 5-15%.

It is to be understood that in the present specification and the appended claims by the term "rubberized fabric" I mean a fabric base material of any desired type, the fibers of which are coated or impregnated with natural, synthetic or reclaimed rubber. By the term "nitrocellulose coat" I mean a nitrocellulose coating composition as described in my above mentioned prior Patent No. 2,326,992 or an equivalent nitrocellulose-containing composition. These compositions may also contain pigments, if desired.

In carrying out my present invention, the above described intermediate coat may be applied to a vulcanized rubberized fabric, and the fabric provided with the intermediate coat is then subjected to drying, for example at 140°-160° F. before the application of the top coat layers. However, rubberized unvulcanized fabrics may also be treated according to my invention by applying intermediate base coat layers to the unvulcanized, rubberized fabric, and subjecting the coated material to heating at temperatures, at which curing of the rubber and drying of the intermediate coat takes place. In general, gradual heating of the coated material to 260° F. and then heating of the same at this temperature for one or several hours is sufficient to effect drying of the varnish and vulcanizing of the rubber.

It will be understood from the above description that my invention is susceptible of numerous modifications, and it is to be understood that I do not limit myself to the above specific examples and details described except as defined in the appended claims.

I claim:

1. As an article of manufacture, a coated flexible fabric sheeting comprising a rubberized fabric base provided with an intermediate coating containing about 15-30% of cellulose nitrate, about 15-30% of a solvent, about 3-8% of dibutylphthalate, about 12-22% of alkyd resins having plasticizing properties, about 2-5% butylstearate, about 10-30% of diluents, about 5-10% of pigments, and about 0.1-0.5% of dioctyl sodium sulfosuccinate, and a final nitrocellulose coating applied to said intermediate coating.

2. As an article of manufacture, a coated flexible fabric sheeting comprising a rubberized fabric base provided with an intermediate coating containing about 15-30% of cellulose nitrate, about 15-30% of a solvent, about 3-8% of dibutylphthalate, about 12-22% of alkyd resins having plasticizing properties, about 2-5% butylstearate, about 10-30% of diluents, about 5-10% of pigments, and about 0.1-0.5% of dioctyl sodium sulfosuccinate, and a final nitrocellulose coating, said final nitrocellulose coating consisting of a cellulose nitrate which is soluble in ethyl alcohol, is dissolved in a mixture of ethyl alcohol with toluene, xylene and butyl alcohol, and a plasticizer selected from the group consisting of blown rape seed oil and blown castor oil, applied to said intermediate coating.

3. As an article of manufacture, a coated flexible fabric sheeting comprising a rubberized fabric base provided with layers of an intermediate coating containing about 15-30% of cellulose nitrate with about 12-22% of alkyd resins having plasticizing properties, the amount of cellulose nitrate in said intermediate coating being greater than that of the alkyd resin, said intermediate coating further containing about 15-30% of a solvent, about 3-8% of dibutylphthalate, about 2-5% butyl stearate, about 10-30% of diluents, and about 5-10% of pigments, said fabric sheeting also comprising layers of a final nitrocellulose coating applied to said intermediate coating.

FELIX J. BELLAC.

REFERENCES CITED

The following references are of record in the file of this patent:

UNITED STATES PATENTS

| Number    | Name             | Date          |
|-----------|------------------|---------------|
| 1,324,154 | Howlett          | Dec. 9, 1919  |
| 2,061,528 | Trolander et al. | Nov. 17, 1936 |
| 2,190,705 | Dreyling et al.  | Feb. 20, 1940 |
| 2,223,575 | Pitman           | Dec. 3, 1940  |
| 2,275,716 | Bachman          | May 10, 1942  |
| 1,818,575 | Parrett          | Aug. 11, 1931 |
| 2,171,389 | Cate             | Aug. 29, 1939 |